

May 9, 1961

P. M. COLE

2,983,028

TUFTED STRUCTURES

Filed June 2, 1959



INVENTOR  
PAUL MORRISON COLE

BY *Raymond E. Blomstedt*

ATTORNEY

1

2,983,028

## TUFTED STRUCTURES

Paul Morrison Cole, Wilmington, Del., assignor to E. I. du Pont de Nemours and Company, Wilmington, Del., a corporation of Delaware

Filed June 2, 1959, Ser. No. 817,585

1 Claim. (Cl. 28—78)

This invention relates to novel tufted structures and more particularly to tufted pile carpets having improved properties and methods of making them.

Carpets are usually constructed by attaching pile to a stiff backing fabric, usually latexed burlap. A cushioning layer is normally positioned beneath the carpet during use to provide softness. The stiffness of the backing fabric, however, prevents the cushioning layer from contributing fully to the compressional properties of the pile, and neither the full value of the pile nor that of the cushioning layer is realized.

It is an object of this invention to provide an improved carpet and other products having a novel tufted structure. Another object is to provide an improved carpet with a greater apparent depth and luxuriosness than conventional carpets while utilizing less pile per unit area. Another object is to provide a process for producing the above products. Other objects will become apparent from a description of the invention given below.

The above objects are accomplished by providing a tufted article comprising a backing member, pile yarn tufted into said backing member, and a bracing web parallel to the backing member and intermediate the backing member and the peaks of the pile yarn and connecting the pile yarn at or below the midpoints in the height of the pile yarn, preferably from  $\frac{1}{3}$  to  $\frac{1}{2}$  the height of the pile.

Figure I illustrates the product of this invention and a procedure for producing it.

The backing member may be any dimensionally stable sheet material including woven, knitted and non-woven fabrics of natural or synthetic fibers, such as burlap, cotton, sisal, wool, rayon, polyamides, polyesters, acrylonitrile polymers and copolymers, vinyl chloride polymers and copolymers, cellulose acetate, glass, metal, paper, and other stabilizing materials such as films, papers, felts, etc.

The bracing web is positioned at the desired distance from the backing member while the tufts of pile yarn are carried through both of these layers. The bracing web serves to hold the pile erect so that the load-bearing ability of the carpet or other structure and the apparent height of the pile are increased. Better compressional properties and aesthetics with less pile yarn are thereby made possible by the novel structure employing the bracing member. This bracing member will usually be a lightweight web which may be a knitted fabric, a woven fabric, or a non-woven fabric or paper.

A lightweight nylon woven marquisette has been found particularly suitable as the bracing member and performs best when treated with a binder to inhibit the stretching of needle holes. The binder may be prepared by making a 5% by weight solution of polyamide resin in methanol. A nylon marquisette as bracing member will give particularly advantageous results when used in the novel structure in combination with a nylon pile yarn. Not only will dyeing problems be simplified but the marquisette

2

web gives strength, mildew resistance, and life comparable to that of the pile yarn.

The pile yarn used in this invention may be either spun yarn or continuous filament yarn, and the fibers, yarns, and fabrics used in the invention may be made from any one of a number of well-known materials such as polyamides (e.g., polyhexamethylene adipamide); copolyamides; polyesters (e.g., polyethylene terephthalate); acrylic polymers and copolymers (e.g., polyacrylonitrile); cellulose derivatives such as cellulose acetate and regenerated cellulose; and the like. Bulked pile yarns are preferred because of better covering properties using less yarn. Suitable bulked yarns may be made according to the methods described by A. L. Breen in U.S. Patent 2,783,609, in U.S. application Serial No. 375,372, filed August 20, 1953, now Patent No. 2,852,906 granted September 23, 1958, by A. L. Breen, and in U.S. application Serial No. 698,103, filed November 22, 1957, by A. L. Breen and H. G. Lauterbach. Other suitable bulked 20 yarns include those commercially available under the names of "Helena," "Banlon," "Fluflon," "Saaba," and the like. Sheath-core yarns can also be used for the pile.

In preparing the novel structures of this invention a conventional tufting machine may be modified to provide an auxiliary needle plate at a predetermined distance from the backing fabric (i.e., the distance from the top of the conventional needle plate to the top of the auxiliary needle plate is set equal to the distance desired between the backing fabric and the bracing web). 25 The auxiliary needle plate supports the bracing web at the desired distance from the backing fabric while the needles of the tufting machine force pile yarn first through the backing then through the bracing web, forming loops on the under side of the bracing web. These loops may 30 be left as such or may be cut in the usual manner. The distance between the bracing web and the backing fabric may be controlled by adjusting the spacing between the auxiliary needle plate and the conventional needle plate.

In addition to employing a single layer as bracing member in the novel structures of this invention, the tufting machine may be accommodated with additional auxiliary needle plates so that two or more bracing webs may be incorporated into the structure. In order to accommodate two or more bracing webs it is usually desirable to provide a higher pile than that used with only one bracing web.

In addition to being useful for carpet structures as described above, the products of this invention may be prepared using alternate structures for additional end uses. For example, a bulked continuous filament nylon may be tufted through a burlap backing and a nylon marquisette fabric in the manner already described, except that the marquisette bracing fabric is positioned at an elevation close to the peaks of the tufts. The 50 product may be dyed and then heat set for 10 minutes in 240° F. steam. Upon removal of the marquisette layer, the product is found to have tufts with tight, well-defined peaks providing a desirable texture of good permanence. The yarn that has been unconfined below the marquisette layer has excellent covering power and satisfactory compressional properties. A similar textured carpet but with greater permanence may be obtained by eliminating the heat setting operation just described and instead applying a 30% by weight solution of polyamide 55 resin in methanol to the tuft peaks. The marquisette layer is then removed after partial evaporation of the methanol.

A carpet may also be prepared with two bracing webs, one at approximately one-half the pile height for improvement of compressional properties, and one located temporarily near the peaks of the tufts in the manner described above in making a textured carpet. These two

bracing webs isolate each tuft of pile yarn from its neighbors and permit the hand printing of colored patterns. The tufts may be properly held in registration to facilitate roller printing of multiple color designs without the diffusion normally associated with such practice. After printing, the top bracing web may be removed and reused.

A Venetian blind may be prepared by tufting widely spaced rows of nylon pile yarn through two bracing webs of nylon marquisette woven fabric held at a distance of three-fourths of an inch apart. Pile loops of minimum size formed on one exterior marquisette fabric are secured, and the pile yarn rows are stiffened by a light application of polyamide resin in methanol. When this structure is positioned with the marquisette bracing webs in a vertical position and the tuft rows in horizontal planes, the product serves as a textile Venetian blind. The pile yarn planes may be tilted by shifting the relative positions of the marquisette webs so as to modify the transmission of light.

An important advantage of this invention is the provision of new carpet and other structures which employ less pile yarn and provide better compressional properties than carpet structures heretofore known. These new structures are cheaper than conventional pile carpets in that less of the most expensive ingredient (i.e., the pile) is employed in their construction. Another advantage is the provision of a carpet structure with a better definition of pile in that each pile yarn has less tendency to mat, as well as a structure which is more adaptable to dyeing and printing when employing nylon in both bracing member and pile yarn. Furthermore, the novel carpet structures exhibit equal recovery from a given load using less pile yarn, compared to commercial samples of tufted carpets.

The novel products of this invention may be used in a variety of applications such as carpeting and rugs, other floor cushioning articles, seat cushioning materials, apparel and industrial fabrics, automobile interior applications, Venetian blinds, and the like.

The following example illustrates specific embodiments of this invention. All parts are by weight unless otherwise specified. The pile yarn illustrated in the example is a bulky continuous filament yarn prepared by the process described by Breen and Lauterbach in U.S. application Serial No. 698,103 filed November 22, 1957. Three ends of 1000 denier/68 filaments of polyhexamethylene adipamide semi-dull luster yarn were used, the filaments of which were drawn 4X and had a Y cross section with a modification ratio of 2.2. This yarn was processed through the jet shown in Figure 7 of that application using steam as the turbulent fluid. The processing conditions for preparing this bulky yarn simulated those used in Run No. 5 in Table V on page 64 of said application. The yarn having a total twist of 0.5 Z is fed to the jet at a speed of 200 yards/minute at a machine overfeed of 72%. The steam passing into the jet was superheated to 600° F. under a steam pressure of 85 p.s.i. The yarn fed to the jet was under minimum tension (i.e., "piddling" tension). The bulky nylon product after tensioning and relaxed boil-off had a yarn denier of 6065.

#### EXAMPLE

Two samples of tufted carpet (A and B) are prepared in accordance with this invention by tufting bulky continuous filament nylon yarn into a lightweight burlap backing and then through a woven nylon marquisette bracing web weighing 0.9 ounce/square yard, employing different weights of pile yarn in the two samples. The bracing web in the carpet is positioned  $\frac{1}{4}$  inch above the backing fabric, and the pile height is approximately  $\frac{1}{2}$  inch above the backing. Two identically constructed conventional tufted carpets (C and D) are prepared as control samples. These controls are made by tufting the same weights of pile yarn into a burlap backing with

out using any bracing web. The four carpet samples are compared using the same Instron compression test. The results given in Table I show that the 14-ounce carpet of this invention has a better set of characteristics than the 19-ounce conventional tufted control sample, made with exactly the same pile yarn. Initial softness in the control sample is exchanged in the tufted sample of this invention for greater thickness, higher recovery, increased compressibility, and improved bottoming effect. Samples A and B also have increased luxuriousness indicated by a higher input of work (i.e., total work of compression) which measurements correlate with subjective appraisals of the four carpet samples. A desirable carpet is one which provides maximum support to the foot or other load applied while the carpet is yielding to the compressive forces of the load. After the application of the initial 6-pound load in the carpet compression test, it is desirable to have a maximum amount of compressibility left for the second compressive cycle. Therefore, the higher the bottoming effect, the better the carpet properties, in the data shown in the table.

Table I

| Sample | Total Carpet Thickness (in.) | Oz. Pile Yarn/Sq. Yd. | Bottoming Effect (in.) | Work of Compression (in. lbs./sq. in.) |
|--------|------------------------------|-----------------------|------------------------|----------------------------------------|
| A      | 0.560                        | 19                    | 0.034                  | 0.707                                  |
| B      | 0.540                        | 14                    | 0.034                  | 0.722                                  |
| C      | 0.542                        | 19                    | 0.024                  | 0.628                                  |
| D      | 0.492                        | 14                    | 0.024                  | 0.552                                  |

The carpet properties reported in the above examples were all determined by the same carpet compression test. Samples of the carpets are preconditioned at 122° F. for a minimum of two hours and then conditioned at 70° F. and 50% relative humidity for at least 16 hours prior to testing at atmospheric temperature and pressure. The tests are performed using the Instron tester, a constant rate strain tensile tester. A circular steel presser foot ( $\frac{3}{4}$  inch diameter) is attached to a cross head traveling at 0.2 inch per minute. The carpet sample (six inches square) is placed on a compression cell and the load applied to the carpet by the moving presser foot. Compression data are automatically recorded on a graph (i.e., load and distance) and with the utilization of an automatic integrator, the total work of compression (area under loading curve) in inch pounds per square inch of carpet can be calculated using simple conversion factors. In carpet compression characterization, a carpet sample is compressed under a pressure limit of 10 p.s.i. for two successive cycles with a relaxation time of 120 seconds between cycles (time in which carpet is not under any compression). The first cycle is used to condition the sample and the actual characterization test parameters of work of compression and bottoming effect are taken from the second cycle. Using the second cycle the work of compression in inch pounds per square inch of carpet is calculated. Using the second cycle the actual compression of the carpet between 6 p.s.i. and 10 p.s.i. is calculated and reported in inches as the bottoming effect.

#### The claimed invention:

A tufted carpet comprising a backing member in the form of a fabric, a bracing sheet of lightweight nylon woven marquisette impregnated with polyamide resin binder superposed above, substantially parallel to and positioned about  $\frac{1}{4}$  inch above the backing member, and bulked continuous filament nylon pile tufted into the backing member and passing through the bracing sheet at between  $\frac{1}{3}$  and  $\frac{1}{2}$  of the height of the pile tufts, said bracing sheet being resiliently supported solely by said tufts.

References Cited in the file of this patent  
UNITED STATES PATENTS

|           |              |               |
|-----------|--------------|---------------|
| 1,012,356 | Hoff         | Dec. 19, 1911 |
| 2,072,152 | Blake et al. | Mar. 2, 1937  |
| 2,132,530 | Greiser      | Oct. 11, 1938 |

|           |
|-----------|
| 2,719,542 |
| 2,748,446 |

|           |              |
|-----------|--------------|
| MacIntyre | Oct. 4, 1955 |
| Mason     | June 5, 1956 |

## FOREIGN PATENTS

|               |               |
|---------------|---------------|
| Great Britain | June 21, 1886 |
| France        | May 29, 1925  |